

# UNITED STATES PATENT OFFICE.

CYRIL HENRY WHITE, OF COVENTRY, ENGLAND.

## PROCESS FOR THE RECOVERY OF BRASS FROM FOUNDRY ASH AND THE LIKE.

1,309,165.

Specification of Letters Patent. Patented July 8, 1919.

No Drawing.

Application filed December 4, 1918. Serial No. 265,296.

*To all whom it may concern:*

Be it known that I, CYRIL HENRY WHITE, a subject of the King of England, residing in No. 9 Park Road, Coventry, Warwickshire, England, have invented a certain new and useful Process for the Recovery of Brass from Foundry-Ash and the like, of which the following is a specification.

This invention relates to a process for recovering brass from foundry ash and the like which remains in pouring pots and crucibles after the brass has been poured therefrom.

According to this invention the said ash is heated to between 1050° C. and 1250° C. and stirred or kneaded while at that temperature. The ash can be heated in a crucible or suitable furnace, and at a temperature over 1050° C. the mass becomes soft; and when stirred or kneaded the liquid brass agglomerates and collects so that it can be poured into molds. The stirring or kneading should be continued so long as the metal continues to collect. It is desirable to use one or more of the ordinary fluxes such as borax, glass, soda ash, or the like, so these form a fusible slag with the impurities, and

unreduced oxids, and they also act as a liquid seal on the surface of the molten mass, thus reducing oxidation and volatilization losses. The slag thus formed will contain a certain amount of copper and zinc, the former of which can be recovered electrolytically.

An increased yield of brass can be obtained by the use of a suitable reducing agent with the ash, such as charcoal or boron-copper.

What I claim as my invention and desire to secure by Letters Patent is:—

A process for recovering brass from foundry ash and the like which remains in pouring pots and crucibles after the brass has been poured therefrom, consisting in heating the said ash to between 1050° and 1250° C. and stirring or kneading the molten mass.

In testimony whereof I have signed my name to this specification in the presence of two subscribing witnesses.

CYRIL HENRY WHITE.

Witnesses:

ALBERT BROWN,  
N. F. MALTBY.